

March 24, 1936.

J. A. DOLL

2,035,425

TOOTHPICK

Filed Nov. 5, 1935



INVENTOR

*Joseph A. Doll*  
BY  
*Horace F. Knott*

ATTORNEY

## UNITED STATES PATENT OFFICE

2,035,425

## TOOTHPICK

Joseph A. Doll, Mineola, N. Y., assignor, by direct  
and mesne assignments, to Joledo Corporation,  
New York, N. Y., a corporation of New York

Application November 5, 1935, Serial No. 48,297

13 Claims. (Cl. 132—90)

This invention relates to toothpicks. The invention aims more especially to provide an improved toothpick packet in which the toothpicks are protected by a folded cover sheet in the manner of the well known book matches, and which is of comparatively low cost. Features of the invention may, however, be embodied in toothpick assemblies without covers and in single toothpicks.

10 Toothpicks according to the invention are made by coating suitably shaped narrow strips of thin cardboard or other suitable sheet paper with a suitable stiffening material to form on the strip a coating of sufficient thickness and 15 which is hard and somewhat flexible and elastic so that the toothpick thus made will be well suited for its intended purpose. The invention includes a method whereby a desired distribution of the coating material on the pointed paper 20 strip is secured.

In the accompanying drawing which shows illustrative embodiments of the invention:—

Fig. 1 is a view in perspective of a toothpick packet containing an assembly of six toothpicks, 25 the packet being shown opened for removal of a toothpick;

Fig. 2 is a plan view of the unfolded paper blank ready to have the toothpick forming strips coated;

30 Fig. 3 is a longitudinal sectional view on an enlarged scale of the completed packet with the cover portion in its folded closed position;

Fig. 4 is a still further enlarged longitudinal sectional view through one of the toothpicks;

35 Fig. 5 is a transverse sectional view on line 5—5 of Fig. 4;

Fig. 6 is a view similar to Fig. 1 but showing a single pick packet; and

Fig. 7 is a plan view of the paper blank for 40 making the article shown in Fig. 6.

Referring to the drawing, and first to Figs. 1 to 5, the toothpick packet shown in Fig. 1 comprises an assembly of toothpicks 10 secured to and extending in parallel relation from a base portion 11, and a cover sheet including a back panel 12 and a front panel 13, the base portion 11 being secured to the back panel 12. When the packet is closed the base 11 and toothpicks 10 are folded down against the back panel 12 of the cover sheet and the front panel 13 is then folded down over the picks so that the picks are covered and enclosed within and protected by the cover sheet as shown by Fig. 3. Most desirably and as shown, some means is 55 provided for holding the front panel 13 in its

closed position. For this purpose in the preferred construction shown the free edge of the front cover panel 13 is provided with a short tab 14 and the base portion 11 has a slot 15 therein into which the tab is inserted as shown in Fig. 3. 5

The toothpicks 10 and base piece 11 are formed from a sheet of thin cardboard or other suitable paper cut to provide a plurality of narrow pointed strips extending from an uncut portion of the sheet which forms the base piece 11, the narrow strips being coated with suitable waterproof stiffening material to give them the necessary stiffness, slight flexibility, and elasticity which toothpicks should have. The coating extends adjacent to but not beyond the line of connection 10 of the strips with the base piece, leaving uncoated 15 paper at the base of each toothpick so that the pick may be readily torn away from the base piece.

Instead of making the cover panels from a 20 separate sheet of paper or other suitable material to which the picks and base 11 are secured, the picks and base piece and the cover panels are most desirably formed all from a single integral strip of thin cardboard or other paper cut 25 to form a blank of the shape shown by Fig. 2. As shown in this figure, the paper strip is cut at one end to provide a plurality of narrow pointed strips 10a extending from the end of the main or body portion of the strip, and the 30 body portion is scored to locate fold lines as indicated by the dotted lines 20 and 21, line 20 being spaced a short distance from the ends of the cuts between the strips 10a to leave the narrow base portion 11, and the line 21 dividing 35 the main portion of the body portion of the strip into the back cover panel 12 and the front cover panel 13, the tab 14 at the free end of the panel 13 and the slot 15 in the base portion 11 being 40 also provided.

Before the blank is folded the coating 10b is applied to the strips 10a. Most desirably, and in accordance with the invention, this is done by dipping the strips 10a points down into a bath 45 of the coating material, then raising the strips from the liquid slowly so as to avoid leaving an excess of liquid thereon, then quickly turning the blank to a position in which the points of the strips 10a extend substantially vertically upward to allow some of the coating material to 50 flow downwardly away from the points of the strips, and then after a short period, usually two or three seconds with coating material which I have used and which is referred to below, turning the blank to horizontal position and main- 55

taining it in that position until the coating material has set.

It is possible that with a suitable coating material of proper viscosity a satisfactory coating may be obtained with a single dip. I have found it desirable, however, in order to obtain a suitable thickness of the coating over the major portion of the picks, to give them two or three successive dips, allowing the coating to set and 10 harden somewhat between dips. I have also found it desirable to use for the first dip a coating material having considerable "body" and because the coating of such material which I have used is somewhat brittle, to use for the second and third coatings a material which gives a 15 more flexible, elastic and tough coating.

A suitable mixture for the first coating is prepared by dissolving 24 oz. of pyroxylin in a mixture of 38% of butyl acetate, 57% of toluol, 20 and 5% of dibutyl phthalate, sufficient solvent being used to give a gallon of solution, and to such solution adding 8 oz. of ester gum and 1 lb. of zinc oxide. A suitable mixture for the second coating, and for the third coating if the picks are 25 dipped three times, is prepared by dissolving 16 oz. of cellulose acetate in 1 gallon of acetone. The resulting composite coating is waterproof, hard, somewhat flexible, and elastic, and does not readily break or crack in the use of the toothpicks. When the picks are dipped in the 30 way described they have a comparatively thin coating at and close to their points, the coating then increasing gradually in thickness for a distance in the direction away from the point, thus giving the greatest rigidity to the picks where most needed and providing them with the desired comparatively thin pointed ends.

Other coating materials may be used provided they are adapted to form the desired hard semi-flexible and elastic coatings. In the materials referred to above, the dibutyl phthalate and ester gum act as plasticizers for preventing brittleness in coating. Other plasticizers might, of course, be used. The zinc oxide serves primarily as a suitable form of filler to give body to the coating and also serves as a pigment to give the toothpicks a clean, white, pleasing appearance.

Figs. 6 and 7 illustrate a single pick packet according to the invention which is similar to the packet of Figs. 1 to 5 except that it has only a single toothpick 10' and the cover 12', 13' is correspondingly narrow.

In making either the single pick packet or the 55 multiple pick packet, the pointed toothpick forming strips of a plurality of packet blanks may be dipped in one operation before the blanks are cut apart along their side edges.

From the illustrative embodiments shown and 60 described, it will be understood that single toothpicks or toothpick assemblies consisting of a plurality of toothpicks extending from a base portion may be made without any enclosing covering.

65 What is claimed is:

1. A toothpick consisting of a pointed paper strip coated with hard semi-flexible elastic and waterproof material.
2. A toothpick consisting of a pointed paper strip having a coating comprising a cellulose base lacquer containing a mineral filler.
3. A toothpick consisting of a pointed paper strip coated with a cellulose base lacquer containing a plasticizer and a mineral filler.
- 75 4. A toothpick consisting of a pointed paper

strip having applied thereto a coating comprising pyroxylin, zinc oxide and a plasticizer.

5. A toothpick consisting of a pointed paper strip having an inner coating comprising a cellulose base lacquer and a mineral filler and an 5 outer tough flexible and elastic coating of cellulose ester.

6. A toothpick consisting of a pointed paper strip having a coating of hard semi-flexible elastic and waterproof material, the coating on the 10 sides of the strip being comparatively thin at the point and increasing in thickness gradually for a distance in the direction away from the point.

7. A toothpick assembly consisting of a paper sheet cut to form a plurality of pointed strips 15 extending from one edge of a base portion, said pointed strips having a coating of hard semi-flexible elastic waterproof material, the coating extending adjacent to but not beyond the line of connection of the strips with said base portion 20 to enable the strips to be readily torn off.

8. A toothpick packet, comprising a toothpick and a cover therefor formed from a strip of sheet material, the major part of the strip being folded to form front and back cover panels, and 25 the part forming the toothpick having a coating of hard semi-flexible elastic waterproof material and being folded to lie between the cover panels.

9. A toothpick packet, comprising an elongated paper sheet cut to form a plurality of narrow 30 strips at one end, said strips being pointed and coated with hard semi-flexible elastic waterproof material to form toothpicks, the coating extending adjacent to but not beyond the line of connection of the toothpick strips with the body of the 35 sheet to permit the toothpicks to be readily torn off, and the body of the sheet being folded to cover the two sides of the toothpicks.

10. A toothpick packet comprising a paper sheet cut to form a plurality of pointed strips 40 extending from one edge of a base portion, said pointed strips having a coating of hard semi-flexible elastic waterproof material, and a cover sheet connected to said base portion and folded to cover the two sides of the coated strips. 45

11. A toothpick packet, comprising a toothpick and a cover therefor formed from a strip of sheet material, the major part of the strip being folded to form front and back cover panels, the part forming the toothpick having a coating of hard semi-flexible elastic waterproof material and being folded to lie between the cover panels, and means for locking the front cover panel in closed position comprising a slot at the 50 base of the toothpick and a tab extending from the end of the front cover panel to enter said slot.

12. The method of making toothpicks, which consists in dipping a pointed strip of paper into a bath of liquid coating material, withdrawing 60 the strip slowly to avoid the presence of excess coating material on the withdrawn strip, quickly inverting the strip to permit some of the coating material to flow away from the pointed end of the strip, and then bringing the strip into 65 substantially horizontal position and maintaining it in such position until the coating has set.

13. A toothpick packet, comprising an elongated paper sheet cut to form a plurality of narrow strips at one end, said strips being pointed 70 and coated with hard semi-flexible elastic waterproof material to form toothpicks, and the body of the sheet being folded to cover the two sides of the toothpicks.